# EUROPEAN PATENT SPECIFICATION

(11) **EP 1 193 316 B1**
(45) Date of publication and mention of the grant of the patent: **28.03.2007**
(21) Application number: 01307257.4
(22) Date of filing: 28.08.2001
(51) Int. Cl.: C21D 7/13, C22C 19/05, C22C 19/07, C22C 38/58

(54) **Nuclear power plant comprising valves made of corrosion resisting and wear resisting alloy**
Kernkraftwerk mit Ventile aus korrosion und verschleiss widerstehender Legierung
Centrale nucléaire avec vannes d'un alliage résistant à l'usure et à la corrosion

(30) Priority: 28.08.2000 JP 2000263258; 03.08.2001 JP 2001235714
(43) Date of publication of application: 03.04.2002
(62) Divisional of application: 05013331.3
(73) Proprietor: Hitachi, Ltd., Chiyoda-ku, Tokyo 100-8010 (JP); Hitachi Kyowa Engineering Co., Ltd., Hitachi-shi, Ibaraki 317-0072 (JP)
(72) Inventor: Kiyotoki, Yoshihisa, Hitachinaka-shi, Ibaraki 312-0011 (JP); Chiba, Yoshiteru, Hitachi-shi, Ibaraki 316-0025 (JP); Kumagai, Shin, Naka-gun, Ibaraki 319-1111 (JP); Ogawa, Yasuhiro, Choshi-shi, Chiba 288-0043 (JP); Sakamoto, Akira, Mito-shi, Ibaraki 310-0912 (JP); Shinohara, Hiroyuki, 3-13 Towa,Adachi-ku Tokyo 120-0003 (JP)
(74) Representative: Hackney, Nigel John

(56) References cited:
- GB-A- 2 308 625
- US-A- 4 789 412
- PATENT ABSTRACTS OF JAPAN vol. 1995, no. 04, 31 May 1995 (1995-05-31) -& JP 07 016610 A (DAIDO STEEL CO LTD), 20 January 1995 (1995-01-20)
- PATENT ABSTRACTS OF JAPAN vol. 012, no. 155 (C-494), 12 May 1988 (1988-05-12) -& JP 62 267413 A (SUMITOMO METAL IND LTD), 20 November 1987 (1987-11-20)
- DATABASE WPI Section Ch, Week 197918 Derwent Publications Ltd., London, GB; Class M27, AN 1979-34547B XP002184607 -& JP 54 040220 A (FUJI KOGYO-SHO KK), 29 March 1979 (1979-03-29)
- PATENT ABSTRACTS OF JAPAN vol. 018, no. 296 (C-1209), 6 June 1994 (1994-06-06) -& JP 06 057360 A (KUBOTA CORP), 1 March 1994 (1994-03-01)

## Description

The present invention relates to nuclear power plant comprising valves of a corrosion-resisting and wear-resisting alloy.

A valve seat or a sliding part, where a corrosion-resisting and wear-resisting alloy which includes cobalt as a base, which is excellent in corrosion-resisting and wear-resisting capabilities, and has a high degree of hardness, and is added with Cr and/or W, is overlaid to prevent an erosion damage on a valve seat during operation or a galling while a valve is in motion is used for valves such as a safety valve in a plant facility such as a turbine power generating facility.

In late years, hydrogen peroxide solution and the like is introduced to adjust water quality in a plant facility such as a turbine power generating facility. As the result, the amount of dissolved oxygen increases on the down stream of the introduction point, and an erosion damage is generated on eutectic carbide of the corrosion-resisting and wear-resisting alloy, which includes cobalt as a base, is added with Cr and/or W, comprises the eutectic carbide and the base material of a cast structure, and is overlaid on a seat surface of a valve and a sliding face to prevent erosion and a galling.

It is also reported that the base material of the cast structure is detached, thereby generating corrosion after the erosion damage of the eutectic carbide when a flow (such as water flow) is present.

The reports relevant to the earlier report include "Thermal and Nuclear Power Vol. 30-5 Processing Method for Boiler Water with Oxygen and Ammonia in a Steam System in a Thermal Power Plant", "Damage on Machinery 1982 2 VEW Operation Experience in a Combined Operation Method at Gerstein Power Generating Plant", and "Materials and Environment Vol. 47, No.3, Effect of Heat Treatment Condition on Grain Boundary Erosion at Welded Part of Cobalt-Base Alloy".

Those reports conclude that there is no effective mean to eliminate a generation of the erosion, and it has been a problem.

On the other hand, an expansion valve preventing a generation of erosion at a valve port provided with an orifice by integrating an orifice member made of a metal material with higher degree of hardness (150 to 500 in Vickers hardness) than that of a valve body with the valve body is disclosed in Japanese application patent laid-open publication No. Hei 08-334280 (corresponding to US patent No. 6164624 Specification).

An increased wear-resisting capability of a blade by attaching a bar-like wear-resisting material including cobalt, nickel, tungsten, manganese, and selenium to a rear edge of the steam turbine blade with friction surfacing is disclosed in Japanese application patent laid-open publication No. Hei 05-208325 (corresponding US patent No. 5183390 Specification). It is disclosed that a caution should be paid to avoid the bar-like wear-resisting material from presenting melting in terms of preventing a change in the degree of hardness and a crack due to shrinkage when the wear-resisting material is attached to the blade by friction surfacing,

A valve where a valve seat comprising 30 to 45 weight % of Cr, 3.0 to 8.0 weight % of Ti, 0 to 10 weight % of Mo, and the balance Ni is diffusion-bonded to a valve element and a valve casing is disclosed in Japanese application patent laid-open publication No. Sho 59-179283.

A valve where a valve seat comprising 10 to 45 weight % of Cr, 1.5 to 6 weight % of at least either of Al or Ti, and 20 weight % or less of Mo, and the balance Ni is diffusion-bonded to a valve element and/or a valve casing is disclosed in Japanese application patent laid-open publication No. Sho 60-86239.

A valve where a valve seat comprising a cemented carbide material or a heat-resisting material is brazed through an amorphous alloy layer to a valve seat part of a valve casing is disclosed in Japanese application patent laid-open publication No. Hei 4-19476.

A technique where material of high carbon martensitic stainless steel is made into an intermediate material with an intermediate dimension with hot plastic forming, the intermediate material is applied with cold plastic forming, and the intermediate material is applied with the hot plastic forming again at 850°C to obtain a steel material with an intended dimension is disclosed in Japanese application patent laid-open publication No. Hei 7-16610. The average dimension of the eutectic carbide in the steel material with the intended dimension reaches 4.2 micrometer with the disclosed technique in the publication.

Valves including safety valves used for a turbine power generating plant have a high flow speed at a valve seat during operation. Cobalt has a high degree of hardness, and is excellent in corrosion-resisting and wear-resisting capabilities. A valve seat which is made of a corrosion-resisting and wear-resisting alloy including cobalt as a base added with Cr and/or W is used for these valves.

A valve casing where the corrosion-resisting and wear-resisting alloy is used on a guide face for guiding a valve element, and on an inner face of a cage to prevent a galling while a vale is in operation, is used for a cage valve.

However, when the aforementioned valve seat made of the corrosion-resisting and wear-resisting alloy is used in a high temperature/high pressure water/steam atmosphere with high dissolved oxygen, a base material layer of a cast structure and eutectic carbide surrounding the base material layer of the cast structure as a mesh shape in the alloy are selectively corroded by the dissolved oxygen in the fluid. This makes the surface of the valve seat rougher, the eutectic carbide is corroded and detached with an additional effect of a tunnel effect (F. j. Heymann: Machine Design. 42, 118 (1970)), which is caused by a penetration of a high speed jet into a corroded and damaged part, the base material of the cast structure which lost the support from the mesh-like eutectic carbide is easily detached by the flow, resulting in a generation of an erosion in the corrosion-resisting and wear-resisting alloy.

Another example of the prior art is US5651842, which discloses a high-speed steel member, and manufacturing method thereof, which member exhibits high toughness, and a hardness of HRC 60 or more. In particular, the high-speed steel member is said to be useful for plastic working.

Another piece of prior art describing a method of working an alloy is JP-A-62267413, which discloses a cast iron containing a eutectic carbide network that is heated to approximately the solidus line temperature plus 80°C and which is held there for 1 to 100 hours. The heat treatment is said to change the shape of the eutectic carbide network, resulting in improved wear and heat check resistances.

JP-A-54040220 discloses an alloy with improved seizing resistance, by increasing the carbon content of the alloy; also disclosed is the addition of chromium which is said to improve the corrosion-resistance of the alloy. The network of carbide that is formed is said to reduce the heat impact resistance of the alloy, and the addition of vanadium is said to convert network eutectic carbides to granular shape.

A gas turbine nozzle formed by casting of an alloy is disclosed in US4789412, which also discloses a method of making a cobalt-based alloy having a eutectic carbide structure, providing high temperature strength and resistance to fatigue caused by thermal stress, due to thermal cycling.

Preferably, the purpose of the present invention is to provide a corrosion-resisting and wear-resisting alloy with increased corrosion-resisting and erosion-resisting capabilities by restraining continuing corrosion of eutectic carbide in the corrosion-resisting and wear-resisting alloy in an atmosphere with dissolved oxygen. Preferably, the purpose of the present invention is also to provide devices where the corrosion-resisting and wear-resisting alloy with increased wear-resisting and corrosion-resisting capabilities is used at wear-resisting parts and erosion-shield parts.

The present invention provides a nuclear power plant as defined in each of claims 1 to 3.

The principal part of the present invention to attain the purpose is described below.

A corrosion-resisting and wear-resisting alloy is obtained by selecting a material from cobalt base added with Cr and/or W, nickel base added with Fe and/or Cr, and iron base added with Cr and/or Ni, casting the material into an ingot or a slab as an intermediate material, applying hot plastic forming at a temperature which is 650°C or more and the solidus temperature or less to the intermediate material, which includes a structure comprising mesh-like eutectic carbide and a base material surrounded by it, forming the eutectic carbide as a discontinuous distribution in a form of multiple grains or clusters. The coefficient of friction of the corrosion-resisting and wear-resisting alloy is 0.1 to 0.5, and the Vickers hardness without age hardening process of it is 300 to 600 Hv.

The cobalt base added with Cr and/or W comprises 0.1 to 3.5% of C, 25% or less of Ni, 25 to 35% of Cr, 5% or less of Fe, 20% or less of W, 1.5% or less of Mn, and 1.5% or less of Si in weight ratio, the balance Co and inevitable impurities. The nickel base added with Fe and/or Cr comprises 0.1 to 2.5% of C, 3 to 9% of Si, 7 to 25% of Cr, 0.5 to 5% of B, 2 to 6% of Fe, 1 to 5% of W, and 17% or less of Mo in weight ratio, the balance Ni and inevitable impurities. The iron base added with Cr and/or Ni comprises 0.1 to 1.5% of C, 0.3 to 4% of Si, 4 to 9% of Ni, 3% or less of Mo, 6 to 10% of Mn, and 15 to 25% of Cr in weight ratio, the balance Fe and inevitable impurities.

For example, cobalt base added with Cr and/or w is cast into an intermediate material typified by an ingot or a slab. This cast material comprises a base material and eutectic carbide of a cast structure. A hot plastic forming is applied to the eutectic carbide, which has a high degree of hardness and low ductility, and is fragile and distributed continuously as a mesh. The intermediate material becomes fine grains or clusters. The structure of the base material penetrates into gaps generated in the eutectic carbide. The base material with a low degree of hardness, high ductility, and strength is distributed around the grain-like or cluster-like eutectic carbide, thereby making the eutectic carbide discontinuous.

Simultaneously, the diffusion of large amount of chrome existing in the eutectic carbide is accelerated by maintaining it at 650°C or more, thereby reducing chrome-deficiency layers around the eutectic carbide, resulting in a corrosion-resisting and wear-resisting alloy simultaneously having an increased corrosion-resisting capability of the eutectic carbide.

With this, eutectic carbide, which is distributed as mesh, and is in a cast structure which is made by dissolving cobalt as a base along with Cr and/or W and comprises the base material and the eutectic carbide, is made into multiple clusters and grains as discontinued eutectic carbide, thereby making an erosion phenomenon discontinued, very shallow and partial.

As the result, the progress of the erosion is restrained, and a tunnel effect (F. j. Heymann: Machine Design. 42, 118 (1970)), which is caused by a penetration of a high speed jet into a corroded and damaged part is restrained, thereby increasing the erosion/corrosion-resisting capability.

The effect described above increases the erosion-resisting and corrosion-resisting capabilities.

Also, the diffusion of large amount of chrome existing in the eutectic carbide into the periphery of the eutectic carbide is accelerated by maintaining it at 650°C or more, thereby reducing chrome-deficiency layers around the eutectic carbide containing Cr, resulting in a corrosion-resisting and wear-resisting alloy simultaneously having an increased corrosion-resisting capability of the eutectic carbide.

For a nickel base material added with Fe and/or Cr, or an iron base material added with Cr and/or Ni, a corrosion-resisting and wear-resisting material is obtained in the same way, thereby increasing erosion/corrosion-resisting capability.

When the corrosion-resisting and wear-resisting alloy is partially or entirely melted, the eutectic carbide at the melted part forms mesh-like eutectic carbide with a low corrosion-resisting capability. Thus, the corrosion-resisting and wear-resisting alloy is machined into an arbitrary shape, and is used after it is joined without melting to a base metal, which is a base to which the corrosion-resisting and wear-resisting alloy is attached.

Since the mesh-like eutectic carbide does not exist, and is made into clusters or grains, a fluid machine using the alloy such as a pump, a valve, a pressure device, and a turbine presents high corrosion/erosion-resisting capabilities under a corrosive atmosphere.

A dynamic machine such as a pump, a valve, a turbine, and an engine where the corrosion-resisting and wear-resisting alloy without chanting the metal composition is joined to a base metal and used for a sliding part or a contact part, presents high corrosion/erosion-resisting capability under a corrosive atmosphere.

The obtained coefficient of friction can be 0.1 to 0.3, which is as low as diamond (coefficient of friction of 0.1 when no lubricant), sapphire (coefficient of friction of 0.2 when no lubricant), and ruby, thereby reducing friction resistance compared with 0.35 to 0.8 of other metals such as brass (coefficient of friction of 0.35 when no lubricant) and steel (coefficient of friction of 0.8 when no lubricant).

The corrosion-resisting and wear-resisting alloy is used for a wear-resisting part or an erosion shield for a fluid machine, and a sliding part or a contact part for a dynamic machine.

When the corrosion-resisting and wear-resisting alloy used in the present invention is attached to a fluid machine or a dynamic machine, it is attached to the wear-resisting part and the erosion shield part, and the sliding part and the contact part while maintaining the composition of the corrosion-resisting and wear-resisting alloy as much as possible. As the attaching method, a joining method which does not melt the corrosion-resisting and wear-resisting alloy is employed. As an example of the joining method, liquid phase diffusion welding is available.

More specifically, the corrosion-resisting and wear-resisting alloy is applied to a valve seat attached to contact faces of a valve element and a valve casing provided on a piping system in an atomic power generating plant and the like, a contact face material for at least either of contact faces of a seat or a washer rotating relatively to each other about a rotating shaft of a pump.

The present invention reduces the degradation of entire corrosion-resisting and wear-resisting capabilities caused by corrosion and damage to eutectic carbide in a corrosion-resisting and wear-resisting alloy.

Applying the corrosion-resisting and wear-resisting alloy of the present invention to sliding parts and contact parts of different devices reduces roughness on the sliding parts and the contact parts of the devices caused by the corrosion and the damage of the eutectic carbide under a corrosive environment, thereby maintaining proper friction resistance on the sliding parts and the contact parts. As the result, the present invention provides devices including sliding faces and contact faces with low friction.

A rotating device, which is an embodiment of the present invention, includes a mechanical seal device sealing between a rotating shaft and a casing. The mechanical seal device comprises a first seal, which rotates with the rotating shaft, and a second seal, which is installed on the casing, and is in contact with the first seal. At least either the first seal or the second seal is a corrosion-resisting and wear-resisting part where grain-like or cluster-like eutectic carbide is diffused in the matrix part of the metal micro structure, and includes the corrosion-resisting and wear-resisting alloy part which comes in contact with the other seal part, and a main body. The corrosion-resisting and wear-resisting alloy part is diffusion-welded to the main body. Since the seal part includes the corrosion-resisting and wear-resisting alloy part, which is diffusion-welded to the main body, the corrosion-resisting and wear-resisting alloy part, which is diffusion-welded, includes grain-like or cluster-like eutectic carbide as described before, not mesh-like eutectic carbide. Seizure, wear, and acceleration of corrosion of the seal member caused by an increase of the temperature at the seal due to heat generated at the contact part of the first and the second seals is restrained, thereby increasing the corrosion-resisting and wear-resisting capabilities at the seal, decreasing the frequency of maintenance for the mechanical seal device including the first and second seals, and increasing the life of the mechanical seal device. This leads to relieving the maintenance operation for the rotating device. Since the corrosion-resisting and wear-resisting alloy has a small coefficient of friction, the heat energy generated at the contact part of the first seal and the second seal decreases. This leads to a reduction of the power rotating the rotating shaft of the rotating device.

### BRIEF DESCRIPTION OF THE DRAWINGS

FIG.1 is an SEM photograph indicating a metal structure of a surface of a corrosion-resisting and wear-resisting alloy including cobalt as a base added with Cr and/or W (a), and its schematic (b).
FIG.2 is an enlarged part (a) of the metal structure of the corrosion-resisting and wear-resisting alloy from Figure 1, and its schematic (b).
FIG.3 is a metal structure indicated by a face analysis of a surface of a corrosion-resisting and wear-resisting alloy including cobalt as a base added with Cr and/or W (a), and its schematic (b).
FIG.4 is a metal structure of a surface of a corrosion-resisting and wear-resisting alloy including cobalt as a base added with Cr and/or W after heat plastic forming (a), and its schematic (b).
FIG.5 is a metal structure indicated by a face analysis of a surface of a corrosion-resisting and wear-resisting alloy including cobalt as a base added with Cr and/or W after heat plastic forming (a), and its schematic (b).
FIG.6 is a schematic of a repeated progress of a damage caused by dissolved oxygen on a corrosion-resisting and wear-resisting alloy including cobalt as a base added with Cr and/or W.
FIG.7 is a schematic of a restraining status of a damage caused by dissolved oxygen on a corrosion-resisting and wear-resisting alloy including cobalt as a base added with Cr and/or W after heat plastic forming.
FIG.8 is a SEM photograph indicating a metal structure obtained by a Strauss test applied to a corrosion-resisting and wear-resisting alloy including cobalt as a base added with Cr and/or W after heat plastic forming.
FIG.9 is a chart indicating a coefficient of friction obtained by a sliding test applied to a corrosion-resisting and wear-resisting alloy including cobalt as a base added with Cr and/or W after heat plastic forming.
FIG.10 is a piping system diagram of a nuclear power generating plant.
FIG.11 is a lengthwise section view of a gate valve adopted for the piping system of the nuclear power generating plant
FIG.12 is a section view indicating contact states between a valve element and individual valve seats, and between a valve casing and the individual valve seats for the gate valve in Figure 11.

### DESCRIPTION OF THE PREFERRRED EMBODIMENT

A typical SEM photograph of a surface of a corrosion-resisting and wear-resisting alloy including cobalt as a base added with Cr and/or W is shown in Figure 1 (Note that (a) is an SEM photograph, (b) is the schematic of (a). Same arrangement is repeated in Figures 2 to 5). An SEM photograph with a high magnitude is shown in Figure 2. An SEM photograph for Cr face analysis taken at the same position on the face of the corrosion-resisting and wear-resisting alloy as in Figure 2 is shown in Figure 3.

An SEM image of a metal structure of a face of the corrosion-resisting and wear-resisting alloy after hot plastic forming such as forging and rolling is shown in Figure 4. An SEM photograph for Cr face analysis taken at the same position on the face of the corrosion-resisting and wear-resisting alloy as in Figure 4 is shown in Figure 5.

Eutectic carbide 1 with principal components of Cr and C in Figures 1, 2, and 3 is continuously distributed as a mesh in a base material 2 of a cast structure including cobalt as a principal component on a surface of the surface-melted alloy.

An embodiment of the present invention is shown in Figures 4 and 5. The eutectic carbide 1 is distributed as grains or clusters with respect to the base material 2 uniformly but discontinuously on a surface of the corrosion-resisting and wear-resisting alloy. The eutectic carbide 1 changes from mesh to grains or clusters, thereby reducing the ratio of the eutectic carbide occupying the surface.

Figure 6 is a schematic showing a progress of repeated damage to the corrosion-resisting and wear-resisting alloy including cobalt as a base added with Cr and/or W due to dissolved oxygen.

As the corrosion/erosion on the corrosion-resisting and wear-resisting alloy progresses, the base layer 2 of the cast structure tends to detach because the dissolved oxygen corrodes the eutectic carbide 1.

As indicated in the SEA photograph in Figure 3, the eutectic carbide 1 continuous as a mesh exists in the conventional corrosion-resisting and wear-resisting alloy including cobalt as a base added with Cr and/or W. The corrosion of the eutectic carbide 1 and the detaching of the base layer 2 of the cast structure due to the dissolved oxygen occur continuously, resulting in a progress of the corrosion/erosion under an atmosphere of dissolved oxygen.

On the other hand, in the corrosion-resisting and wear-resisting alloy which includes cobalt as a base added with Cr and/or W, and is applied with hot plastic forming, the eutectic carbide 1 exists discontinuously as grains or clusters, the corrosive damage to the eutectic carbide 1 due to the dissolved oxygen is limited to the eutectic carbide 1 on a face facing to the dissolved oxygen.

After the eutectic carbide 1 on the surface is corroded and detached, the corrosive damage does not progress any further. This is described using a schematic in Figure 7 showing a restrained damage due to the dissolved oxygen.

To verify the effect described before, JIS G 0575 "Sulfuric acid/cupric sulphate corrosion test on stainless steel" (Strauss test) is applied. According to a test conducted by Takahisa and Honda where a similar test was applied to a corrosion-resisting and wear-resisting alloy of cobalt base including a mesh-like continuous distribution of eutectic carbide (Materials and Environment Vol. 47, No.3, Effect of Heat Treatment condition on Grain Boundary Erosion at Welded Part of Cobalt-Base Alloy), it is reported that a progress of a corrosion is observed at surface-melted alloy of the corrosion-resisting and wear-resisting alloy of cobalt base.

The similar test is applied to the corrosion-resisting and wear-resisting alloy of cobalt base added with Cr and/or W after a plastic forming such as forging and rolling, little etching was observed on the surface, no progress of a corrosion is present into the depth direction, and an excellent corrosion-resisting capability is confirmed. The test result is presented in Figure 8 and Table 1. Figure 9 shows a measuring result of the coefficient of friction with respect to the increase/decrease of the number of sliding.

**TABLE 1**

| Strauss test: Corrosion depth in Co-base alloy (mm) | | | |
|---|---|---|---|
| Material | Co-base alloy with eutectic carbide with continuous mesh-like distribution | Co-base alloy with eutectic carbide with discontinuous grain- or cluster-like distribution | |
| Pre-heating temperature | 600°C | 600°C | 700°C |
| Testing period 16 hours | 0.51 to 0.62 mm | As slight as etching (impossible to measure) | No damage |
| Testing period 150 hours | 3 mm or more | Up to 0.1 mm | As slight as etching (impossible to measure) |

The corrosion depth under a corrosive environment for the corrosion-resisting and wear-resisting alloy of cobalt base added with Cr and/or W, where the eutectic carbide 1 is distributed discontinuously as grains or clusters, the corrosion depth is restrained to about 1/30 of that of conventional alloys, and the corrosion depth is restrained further by increasing a pre-heating temperature to diffuse Cr further.

As the result, the corrosion-resisting and wear-resisting alloy with the eutectic carbide 1 distributed discontinuously as grains or clusters restrains the corrosion due to the dissolved oxygen, resulting in restraining the erosion.

When the cases where pre-heating temperature of the corrosion-resisting and wear-resisting alloy of cobalt base added with Cr and/or W is about 600°C and is 700°C are compared, the corrosion-resisting capability of the grain-like or cluster-like eutectic carbide 1 presents higher corrosion-resisting capability in the case for 700°C, where Cr diffuses more, and joining the alloy with the base material at a higher pre-heating temperature provides better corrosion-resisting and wear-resisting capabilities.

For a corrosion-resisting and wear-resisting alloy of nickel base added with Fe and/or Cr, and a corrosion-resisting and wear-resisting alloy of iron base added with Cr and/or Ni, conducting heat plastic forming in a state heated up to the solidus temperature or less increases the corrosion-resisting and wear-resisting capabilities as for the corrosion-resisting and wear-resisting alloy of cobalt base added with Cr and/or W, simultaneously providing a sliding surface with a low friction.

For a corrosion-resisting and wear-resisting alloy of iron base added with Cr and/or Ni, conducting heat plastic forming in a state heated up to the solidus temperature or less increases the corrosion-resisting and wear-resisting capabilities as for the corrosion-resisting and wear-resisting alloy of cobalt base added with Cr and/or W, simultaneously providing a sliding surface with a low friction.

The material components of the corrosion-resisting and wear-resisting alloy of cobalt base added with Cr and/or w comprises 0.1 to 3.5% of C, 25% or less of Ni, 25 to 35% of Cr, 5% or less of Fe, 20% or less of W, 1.5% or less of Mo, and 1.5% or less of Si in weight ratio, the balance Co and inevitable impurities.

The material components of the corrosion-resisting and wear-resisting alloy of nickel base added with Fe and/or Cr comprises 0.1 to 2.5% of C, 3 to 9% of Si, 7 to 25% of Cr, 0.5 to 5% of B, 2 to 6% of Fe, 1 to 5% of W, and 17% or less of Mo in weight ratio, the balance Ni and inevitable impurities.

The material components of the corrosion-resisting and wear-resisting alloy of iron base added with Cr and/or Ni comprises 0.1 to 1.5% of C, 0.3 to 4% of Si, 4 to 9% of Ni, 3% or less of Mo, 6 to 10% of Mn, and 15 to 25% of Cr in weight ratio, the balance Fe and inevitable impurities.

Applying a hot plastic forming to these corrosion-resisting and wear-resisting alloys increases the corrosion-resisting and wear-resisting capabilities, simultaneously providing a corrosion-resisting and wear-resisting sliding surface with a low friction.

The average coefficient of friction obtained by measuring friction of a face of the corrosion-resisting and wear-resisting alloy is 0.16 without lubrication in a room atmosphere, and is 0.19 in a saturated steam atmosphere at 288°C. The metal components of the corrosion-resisting and wear-resisting alloy used for the friction measuring are described in Table 2, and the eutectic carbide in the corrosion-resisting and wear-resisting alloy takes a form of discontinuous distribution of multiple grains or clusters.

**TABLE 2**

| Composition | Ni | Fe | Mo | C | si | Cr | Co | W |
|---|---|---|---|---|---|---|---|---|
| Weight % | 2.59 | 2.67 | 0.07 | 1.03 | 0.59 | 29.73 | Balance | 3.86 |

The corrosion-resisting and wear-resisting alloy of the present invention is used for different devices as described below. Figure 10 presents a piping system for a nuclear power generating plant. A large number of gate valves and check valves are installed on a water supplying pipe 11 of the piping system 10. Since the gate valves and check valves installed on the water supplying pipe 11 are smaller than a water-supplying pump 12, individual supplied water heaters 13, 14, and other devices installed in the course of the water supplying pipe 11, and the number of the gate valves and check valves is very large, the graphical representation of the gate valves and the check valves are suppressed.

In the nuclear power generating plant, high temperature and high pressure steam obtained inside a nuclear reactor pressure vessel 16 is introduced into a high pressure turbine 18 through a main steam piping 15. Then the steam exhausted from the high pressure turbine 18 is introduced to a low pressure turbine 19. The rotating forces of these turbines drive a generator 20. The steam which has passed through the high pressure turbine 18 and the low pressure turbine 19 is exhausted from the high pressure turbine 18 and the low pressure turbine 19, and is condensed into water in a main condenser 22 and a gland steam condenser 21. The water is returned to the nuclear reactor pressure vessel 16 through the water supplying system 10 including the gate valves and the check valves in addition to the water supplying pump 12, the individual supplied water heaters 13, 14, and the water supplying pipe 11.

The following section describes an example where the present invention is applied to a gate valve among the valves adopted for the piping of a water supplying system 46.

The Figure 11 shows a lengthwise section of the gate valve installed on the water supplying pipe 11 of the water supplying system 10. As in Figure 12, a ring-like plate 31 made of a cobalt-base alloy is mounted as a valve seat on a valve element 30 side of the gate valve. The ring-like plate 31 made of the cobalt-base alloy is also installed on a slide face of a valve seat 33 of a valve casing 32 side.

The cobalt-base alloy includes 1.0 weight % of C, 30.0 weight % of Cr, and 3.9 weight % of W. Eutectic carbide in the cobalt-base alloy is made into clusters or grains less than 30 micrometer by heat forging or heat rolling the cobalt-base alloy. The cobalt-base alloy plate 31 is joined to the valve seat 33 of the valve casing 32 and a valve seat part of the valve element 30 with liquid phase diffusion welding as indicated in Figure 12.

The valve element 30 of the gate valve takes a disk-like shape, which is thick at the top and thin at the bottom, and is driven upward/downward in association with the upward/downward motion of a valve stem, thereby opening/closing a flow of water or steam flowing into the valve casing 32 in the left/right direction in the Figure.

The following section describes a specific example for installing a ring-like plate made of the cobalt-base alloy 31 to the valve element 30. Protrusions 34 protruding toward left and right is provided by providing steps on the left and the right surfaces of the valve element 30 of the gate valve. An insert material for joining is placed in recessed part which is generated by providing the steps. The ring-like plate 31 with thick ness of about 7 mm is placed on the surface of the insert material for joining such that the plate 31 is engaged with the protrusions 34. Only the insert material for joining is melted to attach the ring-like plate 31 to the valve element 30 with liquid phase diffusion welding.

The insert material used for the liquid phase diffusion welding is an Ni-base alloy including 4.5 weight % of Si and 3 weight % of B, and is fully melted at about 1040°C or more. The condition for the liquid phase diffusion welding is 1100°C for the joining temperature, 1 hour for the maintained period, 1 to 2 mult 10⁻⁴ Torr for the degree of vacuum, and 15 g/cm² for the applied pressure. For the cooling after the joining, about 150°C/h is from 1000°C to 650°C, about 100°C/h is from 650°C to 425°C, and natural cooling with air cooling in room is from 425°C.

A ring-like protrusion 35 is also machined on the valve seat 33. An insert material for joining is placed in a recessed part around the protrusion. The ring-like plate 31 with thick ness of about 7 mm is placed on the surface of the insert material for joining to engage with the protrusion 35. Only the insert material for joining is melted to attach the ring-like plate 31 to a valve seat 7 with liquid phase diffusion welding. The ring-like plate 31, the material for joining, the conditions for the liquid phase diffusion welding, and the cooling condition are the same as those for the joining of the valve element 30 to the plate 31.

The valve element 30, the plate 31 and the valve seat 33 do not melt at the joining temperature of 1100°C. Material of a part of the valve element 30 and the valve seat 33 where the plates 31 are installed is S25C, carbon steel for machine structure. The thermal expansion coefficient of the carbon steel for machine structure S25C is smaller than that of the Co-base alloy. The ring-like protrusions 34, 35 (steps) with the height of 2 mm are provided to internally come in contact with a ring-like plates 6 to be joined on the surfaces of the valve element 30 and the valve seat 33 opposing to each other as described in Figure 12. This facilitates positioning the plates 31 to the valve element 30 and the valve seat 33 during the joining, and simultaneously increasing a resistance against a searing force added to a sliding part and the joined part when the gate vale is in operation.

Both of the plates 31 which serve as a valve seat on the valve element 30 side appear as a ring seen from the left and the right of the page respectively in Figure 12. The ring-like plates 31 are joined such that they are in contact with the outer periphery of the circular protrusion 34 on the left and right sides of the valve element 30.

The valve seat 33 on the side of the valve casing 32 is cylindrical, and a valve set 33 is integrated into the valve casing 32. An end face on the side of the valve element 30 of the valve seat 33 is a sliding face. The end face is structured such that the ring like plate 31 is in contact with and is liquid-phase-diffusion welded to the outer periphery of the ring-like protrusion 35. Both of the protrusions 34, 35 are 2 mm in height, which is smaller than 7 mm of the thickness of the ring-like plates 31.

For the gate valve manufactured with this method, the mutual contact faces of the valve element and the valve casing are structured with the plates 31. Since the eutectic carbide in the Co-base alloy, which is the material for the plate 31, is distributed discontinuously as multiple grains or clusters after the liquid phase diffusion welding, the phenomenon that an atmosphere generating a corrosive environment such as dissolved oxygen corrodes the eutectic carbide continuously is restrained. This restrains the detach of matrix of the cast structure of the Co-base alloy, thereby restraining the progress of the corrosion and erosion of the valve seat, resulting in preventing the deterioration of the leakage-resisting capability of the gate valve.

For this embodiment, the Co-base alloy plates 31 are used as the ring-like corrosion-resisting and wear-resisting alloy. As described before, the corrosion-resisting and wear-resisting alloy of nickel base added with Fe and/or Cr, the corrosion-resisting and wear-resisting alloy of iron base added with Cr and/or Ni, and the Ni-base alloy and the Fe-base alloy, where the alloy including components described before in the Table 2 is applied with heat forging or heat rolling to make the eutectic carbide in the alloy distribute discontinuously are used as well.

Though in this embodiment, Ni-base alloy with a low melting point is used as an insert material, an Fe-base or Co-base insert with a low melting point is used as well. The same constitution as in the embodiment of the present invention can be applied to a sliding part and a contact part of a valve seat and the like in a check valve, a safety valve, and a globe valve in addition to a gate valve to provide an effect on restraining the decrease of the leakage-resisting capability, the controllability and the operation capability of the individual valves.

This embodiment has an effect of maintaining the normal function of a valve used for an atomic power generating plant for a long period, thereby increasing the reliability of the atomic power generating plant with the effect.

In a plant including a piping system integrated with the valve described in this embodiment, corrosion and erosion of sliding parts such as a valve seat due to dissolved oxygen are restrained when hydrogen peroxide solution is infused in the piping for the purpose of adjusting water quality, thereby providing an effect on the increase of the safety of the plant.

Especially, when the valve of the present embodiment is installed and used on a water supplying system of a nuclear power generating plant, corrosion and detaching of the eutectic carbide of the co-base alloy applied to the valve seat, and effusion and diffusion of cobalt into the water supplying system after the corrosion and the detaching are restrained. As the result, the effusion and diffusion of the cobalt and the activation of the cobalt are restrained, thereby remarkably reducing exposure to radiation of workers in the nuclear power generating plant.

## Claims

1. A nuclear power plant, which is provided with a piping system including a valve on a piping through which a coolant flows, wherein said valve is provided with a valve element and a valve casing,
wherein valve seats are provided on contact faces of both of the valve element and the valve casing, and a base body of said valve seats is provided with a member of cobalt-base alloy, in which grain-like or cluster-like eutectic carbide is diffused as a discontinued distribution, and which has the coefficient of friction of 0.1 to 0.3,
wherein the cobalt-base alloy comprises in weight ratio 0.1% to 3.5% of C, 25% or less of Ni, 25% to 35% of Cr, 5% or less of Fe, 20% or less of W, 1.5% or less of Mo, and 1.5% or less of Si, the balance being Co and impurities.

2. A nuclear power plant, which is provided with a piping system including a valve on a piping through which a coolant flows, wherein said valve is provided with a valve element and a valve casing,
wherein valve seats are provided on contact faces of both of the valve element and the valve casing, and a base body of said valve seats is provided with a member of nickel-base alloy, in which grain-like or cluster-like eutectic carbide is diffused as a discontinued distribution, and which has the coefficient of friction of 0.1 to 0.3,
wherein the nickel-base alloy comprises in weight ratio 0.1% to 2.5% of C, 3% to 9% of Si, 7% to 25% of Cr, 0.5% to 5% of B, 2% to 6% of Fe, 1% to 5% of W, and 17% or less of Mo, the balance being Ni and impurities.

3. A nuclear power plant, which is provided with a piping system including a valve on a piping through which a coolant flows, wherein said valve is provided with a valve element and a valve casing,
wherein valve seats are provided on contact faces of both of the valve element and the valve casing, and a base body of said valve seats is provided with a member of iron-base alloy, in which grain-like or cluster-like eutectic carbide is diffused as a discontinued distribution, and which has the coefficient of friction of 0.1 to 0.3,
wherein the iron-base alloy comprises in weight ratio 0.1% to 1.5% of C, 0.3% to 4% of Si, 4% to 9% of Ni, 3% or less of Mo, 6% to 10% Mn and 15% to 25% of Cr, the balance being Fe and impurities.

4. A nuclear power plant according to any one of the preceding claims, wherein the grain size of the eutectic carbide is less than 30 µm.

## Patentansprüche

1. Kernkraftwerk mit einem Rohrleitungssystem, das an einer von Kühlmittel durchflossenen Rohrleitung ein Ventil mit einem Ventilelement und einem Ventilgehäuse aufweist,
wobei an Berührungsflächen von Ventilelement und Ventilgehäuse Ventilsitze vorgesehen sind und ein Grundkörper der Ventilsitze mit einem Bauteil aus einer Kobaltlegierung versehen ist, in der korn- oder klumpenartiges eutektisches Karbid in diskontinuierlicher Verteilung diffundiert ist und das einen Reibungskoeffizient von 0,1 bis 0,3 aufweist,
wobei die Kobaltlegierung in Gewichtsanteilen 0,1% bis 3,5% C, 25% oder weniger Ni, 25% bis 35% Cr, 5% oder weniger Fe, 20% oder weniger W, 1,5% oder weniger Mo und 1,5% oder weniger Si, Rest Co und Verunreinigungen, enthält.

2. Kernkraftwerk mit einem Rohrleitungssystem, das an einer von Kühlmittel durchflossenen Rohrleitung ein Ventil mit einem Ventilelement und einem Ventilgehäuse aufweist,
wobei an Berührungsflächen von Ventilelement und Ventilgehäuse Ventilsitze vorgesehen sind und ein Grundkörper der Ventilsitze mit einem Bauteil aus einer Nickellegierung versehen ist, in der korn- oder klumpenartiges eutektisches Karbid in diskontinuierlicher Verteilung diffundiert ist und das einen Reibungskoeffizient von 0,1 bis 0,3 aufweist,
wobei die Nickellegierung in Gewichtsanteilen 0,1% bis 2,5% C, 3% bis 9% Si, 7% bis 25% Cr, 0,5% bis 5% B, 2% bis 6% Fe, 1% bis 5% W und 17% oder weniger Mo, Rest Ni und Verunreinigungen, enthält.

3. Kernkraftwerk mit einem Rohrleitungssystem, das an einer von Kühlmittel durchflossenen Rohrleitung ein Ventil mit einem Ventilelement und einem Ventilgehäuse aufweist,
wobei an Berührungsflächen von Ventilelement und Ventilgehäuse Ventilsitze vorgesehen sind und ein Grundkörper der Ventilsitze mit einem Bauteil aus einer Eisenlegierung versehen ist, in der korn- oder klumpenartiges eutektisches Karbid in diskontinuierlicher Verteilung diffundiert ist und das einen Reibungskoeffizient von 0,1 bis 0,3 aufweist,
wobei die Eisenlegierung in Gewichtsanteilen 0,1% bis 1,5% C, 0,3% bis 4% Si, 4% bis 9% Ni, 3% oder weniger Mo, 6% bis 10% Mn und 15% bis 25% Cr, Rest Fe und Verunreinigungen, enthält.

4. Kernkraftwerk nach einem der vorhergehenden Ansprüche, wobei die Korngröße des eutektischen Karbids mindestens 30 µm beträgt.

## Revendications

1. Centrale nucléaire, qui présente un système de tuyauterie comprenant une vanne sur une tuyauterie à travers laquelle un agent de refroidissement s'écoule, où ladite vanne est munie d'un élément de vanne et d'un carter de vanne,
où des sièges de vanne sont prévus sur les faces de contact à la fois de l'élément de vanne et du carter de vanne, et un corps de base desdits sièges de soupape présente un élément en un alliage à base de cobalt, dans lequel du carbure eutectique en forme de grains ou en forme d'agglomérats est diffusé selon une distribution discontinue, et qui possède un coefficient de friction de 0,1 à 0,3,
où l'alliage à base de cobalt comprend, en pour cent en poids, 0,1% à 3,5% de C; 25% ou moins de Ni, 25% à 35% de Cr, 5% ou moins de Fe, 20% ou moins de W, 1,5% ou moins de Mo, et 1,5% ou moins de Si, le reste étant du Co et des impuretés.

2. Centrale nucléaire, qui présente un système de tuyauterie incluant une vanne sur une tuyauterie à travers laquelle un agent de refroidissement s'écoule, où ladite vanne est munie d'un élément de vanne et d'un carter de vanne,
où des sièges de vanne sont réalisés sur les surfaces de contact à la fois de l'élément de vanne et du carter de vanne, et un corps de base desdits sièges de vanne présente un élément en un alliage à base de nickel, où du carbure eutectique en forme de grains ou en forme d'agglomérats est diffusé selon une distribution discontinue, et qui possède le coefficient de friction de 0,1 à 0,3,
où l'alliage à base de nickel comprend en pour cent en poids 0,1% à 2,5% de C, 3% à 9% de Si, 7% à 25% de Cr, 0,5% à 5% de B, 2% à 6% de Fe, 1% à 5% de W, et 17% ou moins de Mo, le reste étant du Ni et des impuretés.

3. Centrale nucléaire, qui présente un système de tuyauterie comprenant une vanne sur une tuyauterie à travers laquelle un agent de refroidissement s'écoule, où ladite vanne est munie d'un élément de vanne et d'un carter de vanne,
où des sièges de vanne sont réalisés sur des surfaces de contact à la fois de l'élément de vanne et du carter de vanne, et un corps de base desdits sièges de vanne présente un élément en un alliage à base de fer, dans lequel du carbure eutectique en forme de grains ou en forme d'agglomérats est diffusé selon une distribution discontinue, et qui possède le coefficient de friction de 0,1 à 0,3,
où l'alliage à base de fer comprend en pour cent de poids 0,1% à 1,5% de C, 0,3% à 4% de Si, 4% à 9% de Ni, 3% ou moins de Mo, 6% à 10% de Mn et 15% à 25% de Cr, le reste étant du Fe et des impuretés.

4. Centrale nucléaire selon l'une des revendications précédentes, où la taille des grains du carbure eutectique est inférieure à 30 µm.
